# EUROPEAN PATENT SPECIFICATION

(11) **EP 0 004 191 B1**
(45) Date of publication and mention of the grant of the patent: **05.05.1982**
(21) Application number: 79300369.0
(22) Date of filing: 09.03.1979
(51) Int. Cl.: C25B 1/46

(54) **Chloralkali electrolytic cell and method for operating same**
Chloralkali Elektrolysezelle und Verfahren zu deren Betrieb
Cellule pour l'électrolyse des solutions de chlorure de métal alcalin et procédure de fonctionnement d'une telle cellule

(30) Priority: 13.03.1978 US 885754
(43) Date of publication of application: 19.09.1979
(73) Proprietor: ELTECH SYSTEMS CORPORATION, Boca Raton Florida 33434 (US)
(72) Inventor: LaBarre, Ronald Lowry, Huntington Beach California 92646 (US)
(74) Representative: Cronin, Brian Harold John

## Description

The present invention relates generally to the operation of an oxygen electrode in an electrolytic cell, particularly for the production of chlorine and caustic (sodium hydroxide) in such a manner as to reduce significantly the voltages necessary for the operation of such electrolytic cells and to increase substantially the power efficiencies available from such electrolytic cells utilizing oxygen electrodes. More particularly, the present disclosure relates to improved methods of operation of chlor-alkali electrolytic cells having oxygen electrodes, which include utilizing a positive air to liquid pressure drop on the air feed side of the oxygen electrode to improve performance, control of the total flow of the gas feed stream to improve the mass transfer on the air feed side of the oxygen electrode at the reaction sites, humidification of the gas feed to the oxygen electrode to reduce drying out and delamination of the oxygen electrode, so that it functions at a higher current density over a longer lifetime, and the elimination of certain gases such as carbon dioxide, so as to increase the lifetime of the oxygen electrode by elimination of salts which might be formed upon the porous structure of the oxygen electrode during use. These methods of operation may be utilized singularly or preferably in combination to produce higher power efficiencies at lower voltages so as to produce a more energy- efficient oxygen electrode in an electrolytic cell especially suitable for the production of chlorine and caustic (sodium hydroxide).

Chlorine and caustic are essential large-volume commodities which are basic chemicals required by all industrial societies. They are produced almost entirely electrolytically from aqueous solutions of alkali metal halides, more particularly sodium chloride, with a major portion of such production coming from diaphragm type electrolytic cells. In the diaphragm electrolytic cell process, brine (sodium chloride solution) is fed continuously to the anode compartment to flow through a diaphragm usually made of asbestos particles formed over a cathode structure of a foraminous nature. To minimize back migration of hydroxide ions, the flow rate is always maintained in excess of the conversion rate, so that the resulting catholyte solution has unused or unreacted sodium chloride present. The hydrogen ions are discharged from the solution at the cathode in the form of hydrogen gas. The catholyte solution, containing caustic soda (sodium hydroxide), unreacted sodium chloride and other impurities, must then be concentrated and purified to obtain a marketable sodium hydroxide commodity and sodium chloride which is to be reused in electrolytic cells for further production of sodium hydroxide and chlorine. The evolution of the hydrogen gas utilizes a higher voltage so as to reduce the power efficiency possible from such an electrolytic cell, this creating an energy inefficient means of producing sodium hydroxide and chlorine gas. U.S. Patent Number 3, 926,769 discloses an apparatus and process for the production of chlorine gas and an alakali metal hydroxide in a diaphragm cell, where the diaphragm is a cation exchange material and an oxidising gas of controlled moisture content is supplied so as to contact a foraminous cathode in the cathode compartment during operation of the cell.

With the advent of technological advances such as dimensionally stable anodes and various coating compositions therefore, which permit ever narrowing gaps between the electrodes, the electrolytic cell has become more efficient, in that the power efficiency is greatly enhanced by the use of these dimensionally stable anodes. Also, the hydraulically-impermeable membrane has added a great deal to the use of electrolytic cells in terms of selective migration of various ions across the membrane, so as to exclude contaminants from the resultant product and thereby eliminate some of the costly purification and concentration steps from the later processing stages. Thus, the great advances of the past have tended to improve the efficiency of the anodic side and the membrane or separator portion of electrolytic cells. More attention is now being directed to the cathodic side of the electrolytic cell, in an effort to improve the power efficiency of cathodes utilized in electrolytic cells and thus make significant energy savings in the production of chlorine and caustic. Looking more specifically at the problem of the cathodic side of a conventional chlorine and caustic cell, in a cell employing a conventional anode and cathode separated by a diaphragm, the electrolytic reaction at the cathode may be represented as:

The potential of this reaction versus a standard H₂ electrode is -0.83 volt. Under ideal circumstances, the desired reaction to be promoted at the cathode would be:

The potential for this reaction is +0.40 volt, which would result in a theoretical voltage saving of 1.23 volts. The electrical energy necessarily consumed to produce hydrogen gas, which is produced at the cathode of conventional electrolytic cells, has not been counter-balanced efficiently in industry by the utilization of the hydrogen, since it is basically an undesired product of the reaction. While some uses have been found for this excess hydrogen gas, they do not make up the difference in expenditure of the electrical energy involved in generating the hydrogen; thus, if the evolution of hydrogen could be eliminated, it would save electrical energy and thus make the production of chlorine and caustic a more energy efficient reaction.

The oxygen electrode presents one possibility of elimination of this reaction, since it consumes electro-chemically-activated oxygen, which combines with water and the electrons available at the cathode in accordance with the following equation

It is readily apparent that this reaction is more energy efficient, due to the absence of any production of hydrogen at the cathode and the reduction in potential as shown above. This reaction is brought about by feeding an oxygen-rich fluid such as air or oxygen to the oxygen side of an oxygen electrode, where the oxygen finds ready access to the electrolytic surface and is thus consumed in accordance with the above equation. However, this requires a slightly different structure for the electrolytic cell itself, so as to provide an oxygen compartment on the cathodic side of the cathode, so that the oxygen-rich fluid may be fed thereto.

The oxygen electrode itself is well known in the art, since the many NASA projects set up to promote space travel during the 1960s also provided funds for the development of a fuel cell utilizing an oxygen electrode and a hydrogen anode so that the feeding of hydrogen and oxygen gas would produce an electrical current for utilization in a space craft. While this major governent-financed research effort produced many fuel cell components, including an oxygen electrode, the circumstances and the environment in which the oxygen electrode functioned were quite different from those experienced in a chlor-alkali cell. While much of the technology developed in the NASA projects is of value in the chlor-alkali industry with regard to development of an oxygen electrode, much further development is necessary to adapt the oxygen electrode to the chlor-alkali cell environment.

Some attention has been given to the use of an oxygen electrode in a chlor-alkali cell, so as to increase efficiency in the manner considered to be theoretically feasible, but thus far the oxygen electrode has failed to generate sufficient interest to produce commercially effective or economically viable forms for use in electrolytic cells for the production of chlorine and caustic. While it is recognized that an effective oxygen electrode will be necessary in order to realize the theoretical efficiencies available, the chlor-alkali cell will require operational methodology significantly different from that of a fuel cell, since an electrical potential is applied to the chlor-alkali cell for the production of chlorine and caustic, in addition to the supply of an oxygen-rich fluid to promote the relevant electrochemical reaction. Therefore, it would be advantageous to develop the methodology for the operation of oxygen electrodes specifically so as to maximize the electrical efficiency obtainable with oxygen electrodes in chlor-alkali cells for the electrolytic production of chlorine and caustic.

### Summary of the Invention

According to this invention, a method is provided for operating a chlor-alkali electrolytic cell having an anode compartment, a cathode compartment divided from the anode compartment by a separator and an oxygen compartment divided from the cathode compartment by an oxygen electrode, which method comprises feeding an alkali metal halide solution to the interior of the anode compartment, feeding an aqueous alkaline solution to the interior of the cathode compartment, feeding a gas containing molecular oxygen to the interior of the oxygen compartment, applying an electrical potential between the cathode and the anode, removing halogen gas from the anode compartment, removing alkali metal hydroxide from the cathode compartment and removing an oxygen-depleted gas from the oxygen compartment, characterized in that the gas containing molecular oxygen is depleted of carbon dioxide and humidified and it is fed to the oxygen compartment at a positive gauge pressure in the range from 0.25 to 500 grams per square centimetre (0.1 to 200 inches of H₂0) and so as to provide a total flow rate in excess of the theoretical stoichiometric amount of oxygen necessary for the reaction.

According to a second aspect of this invention, a chlor-alkali electrolytic cell is provided, for the production of chlorine and alkali metal hydroxide, comprising an anode compartment for containing an anolyte comprising an alkali metal chloride, a cathode compartment for containing a catholyte comprising an alkali metal hydroxide, a separator dividing the cathode compartment from the anode compartment, an oxygen compartment for receiving an oxygen-containing gas, means for controlling the moisture content of the oxygen-containing gas, means for controlling the total flow-rate of the oxygen-containing gas within the oxygen compartment, an oxygen electrode dividing the cathode compartment from the oxygen compartment, means for removing chlorine from the anode compartment, means for removing alkali metal hydroxide from the cathode compartment, means for supplying alkali metal chloride to the anode compartment and means for supplying electrolyzing electrical energy to the anode and the cathode, characterized in that the cell includes means for controlling the pressure of the oxygen-containing gas within the oxygen compartment.

According to a preferred feature of the method of the invention, the total flow rate is in the range from 1.5 to 21 times and, most preferably, in the range from 1.5 to 5 times the theoretical stoichiometric amount of oxygen.

The oxygen-containing gas is preferably supplied at a positive gauge pressure in the range from 0.25 to 250 grams per square centimetre (most preferably, from 100 to 200 grams per square centimetre). These ranges are respectively equivalent to, firstly, the range from 2 to 100 inches of H₂0 and, secondly, from 40 to 80 inches of H₂0.

The preferred embodiments of this invention are shown in the drawings and described by way of example in this disclosure without attempting to show all of the various forms and modifications of the invention which are possible.

### Brief description of the drawing

Figure 1 is a schematic view of an electrolytic cell for the production of halogen gas and alkali metal hydroxides according to the present invention;
Figure 2 is a graphical representation of the relationships between total flow, pressure differential and measured potential of the cathode.

### Description of the preferred embodiments

Referring to Figure 1, a monopolar divided electrolytic cell is indicated at 12, which is suitable for use according to the present invention. It is recognized that various other designs of electrolytic cells can operate according to the method of the present invention but, for purposes of illustration, the present schematic view amply allows the details of the invention to be appreciated. The electrolytic cell 12, as shown in Figure 1, would generally have some environmental supporting structure or foundation to maintain it in correct alignment with other like cells, so as to build a bank of electrolytic cells for production purposes. The details of this environmental structure have not been shown, to facilitate illustration of the present invention. The cell itself could be manufactured from various metallic or plastics materials, provided these materials resist the caustic surroundings of the chlorine cell environment and the temperature conditions which arise during the operation of basic chlor-alkali cells, which are well known in the art. Such materials generally include (but are not limited to) metallic materials, such as steel, nickel, titanium and other valve metals, and plastics materials, such as polyvinyl chloride, polyethylene, polypropylene, "Fiberglas" (Regd. Trademark) and others too numerous to mention. The valve metals include aluminium, molybdenum, niobium, titanium, tungsten, zirconium and alloys thereof.

It can be observed from the drawing that the electrolytic cell 12 has an anode 14, a separator 16 and a cathode 18, so that three individual compartments are formed within the electrolytic cell, namely an anode compartment 20, a cathode compartment 22 and an oxygen compartment 24.

The anode 14 generally is constructed of a metallic substance, although graphitic carbon could be used, as in the old electrodes now largely discarded by industry. Anodes for use in the chlor-alkali cell 12 generally are of active materials resistant to the anolyte, such as a valve metal. A preferred valve metal based upon cost, availability and electrical and chemical properties is titanium. Titanium substrates used in the manufacture of electrodes may take a number of forms for example, solid metal sheet, expanded metal mesh, with a large percentage of open area, and porous titanium with a density of 30% to 70% of that of pure titanium, which can be produced by cold compacting titanium powder. Porous titanium is usually the preferred material, because of its long life characteristics and its relative structural integrity. If desired, porous titanium can be reinforced with titanium mesh, e.g. for large electrodes.

Usually these substrate materials carry a surface coating to protect the material against passivation and give a so-called dimensionally-stable anode. Most of these coatings contain a noble metal, a noble metal oxide (either alone or in combination with a valve metal oxide) or other electro- catalytically-active corrosion-resistant materials. Dimensionally stable anodes are well-known and are widely used in the industry. One type of coating is a Beer-type coating, described in U.S. Patent Specfications 3,236,756, 3,623,498, 3,711,385, 3,751,296 and 3,933,616. Another type of coating contains tin, titanium and ruthenium oxides, as described in U.S. Patent Specifications 3,776,834 and 3,855,092. Other examples of surface coatings are one containing tin, antimony and titanium and ruthernium oxides, described in U.S. Patent Specification 3,875,043, and another containing tantalum and iridium oxides, described in U.S. Patent Specification 3,878,083. Of course, other coatings are available, as those skilled in the art will know, for use in chlor-alkali cells as well as in other applications in which electrodes are required for electrolytic reactions.

A number of materials may be used for the separator 16 shown in the drawing. One type of material predicates the use of a substantially hydraulically-impermeable structure, namely a cation exchange membrane, as it is known in the art. One type of hydraulically-impermeable cation exchange membrane which can be used in the apparatus of the present invention is a thin film of fluorinated copolymer having pendant sulphonic acid groups. The fluorinated copolymer is derived from monomers of the formulae: in which the pendant -S0₂F groups are converted to -S0₃H groups, and wherein R represents the group R' being fluorine or a fluoralkyl group having 1 to 10 carbon atoms, Y being fluorine or a trifluoromethyl group and m being 1, 2 or 3; n is 0 or 1; X is fluorine, chlorine or a trifluoromethyl group and X' is X or , wherein a is zero or an integer from 1 to 5.

These monomers result in copolymers having the repeating structural units: and

In the copolymer, there should be sufficient repeating units according to formula (3) above to provide an -S0₃H equivalent weight of about 800 to 1600. Materials having a water absorption of about 25 percent or greater are preferred, since higher cell voltages at any given current density are required for materials having less water absorption. Materials having a film thickness (unlaminated) of about 0.20 mm (8 mils) or more require higher cell voltages, resulting in lower power efficiencies.

Because of the large surface areas of membranes in commercial cells, the substrate film material typically is laminated with and impregnated into a hydraulically-permeable electrically non-conductive inert reinforcing member, such as a woven or non-woven fabric made of fibres of asbestos, glass, .Teflon (Regd. Trademark) or the like. In film/fabric composite materials, it is preferable for the laminating to produce an unbroken surface of the film resin on at least one side of the fabric, to prevent leakage through the substrate film material.

Materials of this type are further described in U.S. Patent Specifications 3,041,317, 3,282,875, 3,624,053 and 3,784,399 and British Patent Specification 1,184,321. Hydraulically-impermeable cation exchange substrate materials comprising fluorinated copolymers having pendant sulphonic groups as aforedescribed, are available from E. I. duPont deNemours and Co. under the trademark Nafion.

Polymeric materials according to formulae (3) and (4) can also be made, wherein other types of ion exchange groups are present, instead of sulphonic acid exchange groups. One particular type of structure is a carboxyl group ending in either an acid, an ester or a salt to form an ion exchange group similar in behaviour to the sulphonic acid. In such a structure, instead of S0₂F, the group COOR² is in its place, wherein R² may be a hydrogen or alkali metal ion or an organic group. These polymeric materials are available from E. I. duPont deNemours Et Co. Furthermore, it has been found that a substrate material such as Nafion (Regd. Trademark) may have any ion exchange group or any functional group capable of being converted into an ion exchange group or into which an ion exchange group can easily be introduced, including oxy acids, salts or esters of carbon, nitrogen, silicon, phosphorus, sulphur, chlorine, arsenic, selenium and tellurium.

A second type of substrate material has a backbone chain of copolymers of tetrafluoroethylene and hexafluoropropylene and, grafted on to this backbone, a 50/50 mixture of styrene and alpha-methyl styrene. These grafts may then be sulphonated or carbonated to obtain the desired ion exchange characteristic. This type of substrate while having different pendant groups has a fluorinated backbone chain, so that the chemical resistivities are reasonably high.

Another type of substrate film material comprises polymeric substances having pendant carboxylic or sulphonic acid groups wherein the polymeric backbone is derived from polyvinyl aromatic and monovinyl aromatic components in an inorganic solvent, under conditions which prevent solvent evaporation and result in a generally copolymeric substance, although a 100 percent polyvinyl aromatic compound may be prepared which is satisfactory.

The polyvinyl aromatic component may be chosen from divinyl benzenes, divinyl toluenes, divinyl naphthalenes, divinyl diphenyls, divinyl-phenyl vinyl ethers, substituted alkyl derivatives thereof such as dimethyldivinyl-benzenes and similar polymerizable aromatic compounds which are polyfunctional with respect to vinyl groups.

The monovinyl aromatic component is generally the impurities present in commercial grades of polyvinyl aromatic compounds, including styrene, isomeric vinyl toluenes, vinyl naphthalenes, vinyl ethyl benzenes, vinyl chlorobenzenes, vinyl xylenes and alpha-substituted alkyl derivatives thereof, such as alpha-methyl-vinyl-benzene. In cases where high-purity polyvinyl aromatic compounds are used, it may be desirable to add monovinyl aromatic compounds so that the polyvinyl aromatic compounds constitute 30 to 80 mole percent of the polymerizable material.

Solvents for dissolving the polymerizable material prior to polymerization are suitable if they are inert to the polymerization (in that they do not react chemically with the monomers or the polymer), have a boiling point greater than 60°C and are miscible with the sulphonation medium.

Polymerization is effected by any of the well-known expedients, for instance, heat, pressure and catalytic accelerators, and is continued until an insoluble, infusible gel is formed substantially throughout the volume of solution. The resulting gel structures are then sulphonated in a solvated condition and to such an extent that not more than 4 equivalents of sulphonic acid groups are formed for each mole of polyvinyl aromatic compound in the polymer and not less than one equivalent of sulphonic acid groups are formed for each 10 moles of polyvinyl and monovinyl aromatic compounds in the polymer. As with Nafion (Regd. Trademark) material, these materials may require reinforcing with similar materials.

Substrate film materials of this type are further described in U.S. Patent Specifications 2,731,408, 2,731,411 and 3,887,499. These materials are available from lonics, Inc. under the trademark Ionics CR6.

Various means of improving these substrate materials have been sought, one of the most effective of which is the surface chemical treatment of the substrate itself. Generally these treatments consist of reacting the pendant groups with substances which will yield less polar bonding and thereby absorb fewer water molecules by hydrogen bonding. This has a tendency to narrow the pore openings through which the cations travel, so that less water of hydration is transmitted with the cations through the membrane. An example of this is to react ethylene-diamine with the pendant groups so as to tie two of the pendant groups together by the two nitrogen atoms in the ethylene-diamine. Generally, with a film thickness of 0.175 mm (7 mils), the surface treatment will be done to a depth of approximately 0.05 mm (2 mils) on one side of the film, by controlling the time of reaction. This results in good electrical conductivity and cation transmission with less hydroxide ion and associated water reverse migration.

The separator 16 may also be a porous diaphragm made of any material compatible with the cell liquor environment, the relevant bubble pressure and electrical conductivity characteristics. One example of such a material is asbestos, which can be used either in paper sheet form or as vacuum- deposited fibres. A further modification can be effected by adding polymeric substances, generally fluorinated, to the slurry from which the diaphragm is deposited. Also, polymeric materials themselves can be made porous to such an extent that they show the operational characteristics of a diaphragm. Those skilled in the art will readily recognize the wide variety of materials which are available for use as separators in chlor-alkali cells.

The third major component of these cells for use according to the methods of the present invention is the cathode 18 shown in the drawing. The cathode 18, in order to be utilized according to the methods of the present invention, necessarily is an oxygen cathode. An oxygen electrode or oxygen cathode may be defined as an electrode which is supplied with a molecular-oxygen-containing fluid in order to lower the voltage below that necessary for the evolution of hydrogen. The basic support for an oxygen cathode generally includes a current collector, constructed for instance of a base metal, although carbon black may also be used. The expression "base metal" is used herein to refer to inexpensive metals which are commercially available for common construction purposes. Base metals are characterized by low cost, ready availability and adequate resistance to chemical corrosion when utilized as a cathode in electrolytic cells. Base metals include, for instance, iron, nickel, lead and tin. Base metals also include alloys such as mild steels, stainless steel, bronze, monel and cast iron. The base metal preferably is chemically-resistant to the catholyte and has a high electrical conductivity. Furthermore, the material is generally slightly porous, such as a mesh, when used in the construction of an oxygen cathode. A preferred metal, based upon cost, resistance to the catholyte and voltages available, is nickel. Other current collectors include tantalum, titanium, silver, gold and plated base metals. One side of this basic support material carries a coating of a porous material, either compacted in such a fashion as to adhere to the nickel or other support or held together with some kind of binding substance so as to produce a porous substrate material. A preferred porous material based upon cost is carbon. Anchored within the porous portion of the oxygen cathode is a catalyst to promote the reaction wherein molecular oxygen combines with water molecules to produce hydroxide groups. These catalysts are generally based upon silver or a platinum group metal, such as palladium, ruthenium, gold, iridium, rhodium, osmium or rhenium, but also may be based upon semiprecious or nonprecious metals, alloys, metal oxides or organometal complexes. Generally such electrodes contain a hydrophobic material in order to wetproof the electrode structure. Of course, those skilled in the art will realize that the porosity of carbon material and the amount and type of catalytic material used will affect the voltages and current efficiencies of the resultant electrolytic cell, as well as their lifetimes. The cathode 18 is preferably constructed according to U.S. Patent Specfication 3,423,247.

As shown in the drawing, the anode 14, the separator 16 and the oxygen cathode 18 divide the electrolytic cell 12 into three compartments, namely the anode compartment 20, the cathode compartment 22 and the oxygen compartment 24. In a chlor-alkali cell an alkali metal halide solution is fed to the andoe compartment 20, by way of an alkali metal halide solution inlet 26. The alkali metal halide solution is preferably one which evolves chlorine gas in use, such as sodium chloride or potassium chloride. The cathode compartment 22 is supplied with an aqueous solution by way of an aqueous solution inlet 28. The aqueous solution must contain sufficient water molecules to be broken down to form the hydroxide groups necessary for the reaction. The oxygen compartment 24 is supplied through an oxygen inlet 30 with a fluid containing a sufficient amount of molecular oxygen to permit operation of the cell as desired. Generally a gas, most preferably air, which has had any carbon dioxide removed and has been humidified or pure molecular oxygen which has been humidified, is used as the fluid. Reaction products such as chlorine gas are removed from the anode compartment 20 through a halogen outlet 32, while aqueous NaOH or KOH is removed from the cathode compartment 22 through an alkali metal hydroxide outlet 34 and an oxygen-depleted fluid, either in the form of residual pure oxygen or air, is preferably removed via a depleted fluid outlet 36.

In using the three compartment cell 12 according to the above description, i.e. as an oxidizing gas depolarized chlor-alkali cell, a pressure differential is applied across the porous cathode 18, so that the pressure in the oxygen compartment 24 is higher than that in the cathode compartment 22. The increased pressure, which may be a zero gauge pressure in order to bubble through but, due to the electrolyte head, may be a negative absolute pressure, assists in mass transfer of the oxidizing gas such as oxygen into the cathode 18 thereby preventing oxygen depletion in the reaction zone within the cathode 18 and leading to a longer lifetime for the cathode. It should be remembered that this pressure differential is based upon the partial pressure of the oxygen present, if less than 100% oxygen is used.

By increasing the total flow of the depolarizing gas in the oxygen compartment 24, the mass transfer of oxygen into the reaction sites within the cathode 18 is also enhanced. This is particularly important when less than 100% pure O2 is used. Molecular oxygen is consumed by the reaction taking place at the catalytic sites within the porous material of the oxygen cathode 18. As oxygen is consumed, additional quantities must become available continuously and must, therefore, be fed continuously into the oxygen compartment 24. The preferred total flow rate is between 1.5 and 10 times the theoretical stoichiometric amount of oxygen necessary for the reaction, a flow rate of about 2.5 times being the best.

Pure oxygen gas may be supplied to the oxygen compartment 24. However, air may also be used, since it contains approximately 23% free molecular oxygen by weight. In the case of air, however, carbon dioxide must be removed before the air is delivered to the oxygen compartment 24. It has been found that carbon dioxide promotes the formation of certain carbonate deposits upon the cathode, which sharply reduce its lifetime and power efficiencies while increasing the voltage. By eliminating the major portion of carbon dioxide from the air, this problem is also largely eliminated.

It has been noticed that the pressure of nitrogen in the air creates problems, since it acts as a diluent and so decreases the concentration of the oxygen present within the oxygen compartment 24 of the electrolytic cell 12. The nitrogen molecules enter the pores of the cathode 18 and must be diffused back out of the pores, since they are not involved in the reaction. This causes a lack of activity within the porous catalytic areas of the oxygen cathode 18, so as to reduce the power efficiency and increase the voltage necessary for the operation of such a cell. It has also been found that this may be reduced to a minimum by increasing the total flow so as to provide an ample oxygen supply to the oxygen compartment 24, thus reducing to a minimum the voltage necessary to operate the cell while increasing to a maximum the possible power efficiency from such an electrolytic cell 12.

It has also been discovered that evaporation and mass transfer pose a problem with the oxygen cathode 18 in the electrolytic cell 12. This problem can be eliminated by increasing the relative humidity of the oxygen or air to be supplied to the oxygen compartment 24, e.g. by bubbling the gas through water at a temperature of 40° to 70°C, so as to produce a relative humidity of approximately 85 percent. This in turn reduces evaporation and also reduces drying out of the cathodes, which can cause delamination of the porous material from the solid support material of the oxygen cathode 18, and so further enhances the mass transfer across the porous surfaces. The gas temperature as fed to the oxygen compartment 24 is generally in the range from 40° to 90°C. and therefore the gas is saturated. Furthermore, humidification seems to have another effect. Mainly, the evaporative driving force which causes mass transfer of the water from the cathode compartment 22 into the cathode structure 18 causes crystallization of the electrolyte and the solids formed reduce seriously the lifetime of a given cathode 18, because they obstruct the pores. Humidification of the feed gas to the oxygen compartment 24 drastically reduces this by eliminating the evaporative driving force involved in transferring the liquid electrolyte from the cathode compartment 22.

However, it has been noted that, if the dew point of the gas feed is higher than the cathode skin temperature, condensation occurs on the cathode surface. When this happens, sites of oxygen mass transfer are occluded, so as to decrease seriously the performance of a given oxygen cathode 18. Therefore, the gas stream dew point is advantageously adjusted to balance these two deleterious effects, so as to maintain the dew point a few degrees below the cathode skin temperature and keep the relative humidity within a range so as to eliminate the evaporative driving force involved. It should be noted that higher operation temperatures lower the voltage of the cell, but may shorten the life of the cathode 18. A temperature in the range of 60° to 85°C. is considered optimum.

In order that those skilled in the art may more readily understand the present invention and certain preferred ways of carrying it into effect, the following specific examples are provided.

### Example 1

An oxygen cathode according to U.S. Patent No. 3,423,247 was installed in an electrolytic cell so that the carbon side faced the oxygen compartment and the nickel side faced the cathode compartment, in which an electrolyte was placed. A dimensionally-stable anode, having a catalytic layer composed of tantalum and iridium oxides, was installed approximately 7 centimetres away from and parallel to the oxygen cathode. A stream of carbon-dioxide-free air was passed into the oxygen compartment of the cell at a flow rate of approximately 790 cubic centimetres per minute, which is approximately 21 times the theoretical stoichiometric amount needed when the cell is operated at a current density of 0.15 amperes per square centimetre (1 ampere per square inch). The pressure in the oxygen compartment was adjusted to approximately 110 grams per square centimetre (44 inches of water) above atmospheric pressure, by restricting the flow from the outlet 36. The pressure was maintained at that level during the test. Electrolyte consisting of approximately 400 grams per litre of NaOH was then added to the cathode compartment 22 and agitated continuously by magnetic stirring apparatus.

The cathode was then conditioned by operating the cell at 60°C. and a current density of approximately 0.05 amperes per square centimetre (1/3 ampere per square inch) for about one day. After conditioning was completed, the current density was increased to approximately 0.15 amperes per square centimetre (1 ampere per square inch). The air flow, pressure, temperature and current density were held constant during the remainder of the test. It should be noted that these tests were used with sodium hydroxide electrolyte only and the cell was not used as a chlor-alkali cell per se. However, the results from these tests correlate closely with those obtained by using chlor-alkali cells, since the type of anode or the spacing of the anode to the cathode are not critical factors, although the anode must be stable in sodium hydroxide solution.

The cathodes were conditioned at the reduced current density because it was thought that the catalytic platinum layer becomes partially oxidized, during the period when the cathodes are stored before use. The conditioning process restores the catalytic layer to high activity without causing deterioration in the quality of the cathode. Slow break-in for less noble catalysts may be harmful, however.

The electrical connection was made on the nickel side of the cathode because it is easier to make a good electrical contact on nickel than on carbon. The cathode reference voltage, measured versus a mercury/mercuric oxide reference electrode cell, changed from -0.31 on day 1 to -1.03 on day 98, when the test was considered completed. The lifetime of this cathode under these test conditions was 2350 hours.

### Example 2

A cathode test was done as described in Example 1, except that the air flow rate was reduced from 790 to 220 cubic centimetres per minute (approximately 6 times the theoretical stoichiometric amount necessary for reaction). The reference voltage changed from -0.43 on day 1 to -2.27 on day 52. The cathode lifetime was 1240 hours in this test, as compared to 2350 when increased air flow was used in Example 1. This shows that, when the total flow increases, the potentials are lower and the life-times are extended.

### Example 3

A cathode test was done as described in Example 1, except that an oxygen flow rate of 150 cubic centimetres per minute was used instead of an air flow rate of 790 cubic centimetres per minute. This oxygen flowrate was about 19 times the theoretical stoichiometric flow required at 0.15 ampere per square centimere (1 ampere per square inch) current density for operation of a cell. For this test, the electrical connection was made on the carbon side of the cathode. The cathode was conditioned by running the cell at a current density of 0.05 amperes per square centimetre (1/3 ampere per square inch) for about 24t hours, then increasing it to 0.1 ampere per square centimetre (2/3 ampere per square inch) for about 24 hours and finally increasing it to about 0.15 ampere per square centimetre (1 ampere per square inch), at which level it was held for the remainder of the test. The reference voltage changed from -0.38 on day 2 to -0.42 on day 293. The test was discontinued on day 293 because delamination of the cathode occurred. The cathode lifetime was about 7030 hours. This again shows that when the total flow is increased, in terms of stoichiometric amounts of available oxygen, the life is extended at lower potentials.

### Example 4

An oxygen cathode test was done according to Example 1, with an operating temperature of approximately 85°C at a current density of approximately 0.3 amperes per square centimetre (2 amperes per square inch), using an NaOH solution of 300 grams per litre. Furthermore, the membrane utilized in the subject test was a standard Nation (Regd. Trademark) film. This experimental cell was operated using various types of cathodes. Comparative cell voltages for the different cathodes were obtained as follows:

As can be seen from the results above, each of these cathodes when compared to a standard hydrogen-evolving steel-mesh cathode shows superior performance utilizing the methods of the present invention.

### Example 5

An oxygen cathode test was done according to Example 1, using air which had not been scrubbed free from carbon dioxide. The cathode was broken in on oxygen and then switched to air. Failure occurred less than 48 hours after switching to air. This performance was typical of cathodes supplied with air which contained carbon dioxide, thus showing the necessity of removing carbon dioxide for the lifetime of an oxygen cathode. The basic conditions were the same as those according to Examples 1-3 and the table below shows the cell voltages and reference voltage, along with remarks.

### SEP vs Hg/HgO

### Examples 6 to 12

Oxygen cathode tests were done according to Example 1 wherein the total air flow rate was varied according to Figure 2 of the drawings and the pressure was also varied. As shown in Figure 2, the cathode potential decreased with increasing flowrates and also decreased with increasing pressures. In each case, the air supplied was free from carbon dioxide and was humidified.

The cathode tests given in the Examples above were ended in each case when the reference voltage reached -1.00 or when delamination of the various layers of the cathode occurred. The air (or oxygen) flow was recorded on cathode life cell test data sheets as the height (in millimetres) of the steel ball on the Matheson 601 flow meter (except for Example 3, where a Matheson 602 flow meter was used). These readings were then converted into cubic centimetres per minute by referring to the appropriate calibration curves. The Examples give the results of cathode tests where pressure differentials were approximately 100 grams per square centimetre (40 inches of water). The term "pressure differential" means the net pressure exerted between the two sides of the cathode. In this case, the difference between the pressure and the oxidizing gas compartment (100 grams per square centimetre above atmospheric pressure) and the average hydrostatic pressure exerted by the electrolyte on the other side of the cathode (10 grams per square metre) is approximately 100 grams per square centimetre. The hydrostatic pressure is calculated by multiplying the density of the electrolyte (1.33) by the average height above the cathode, which was 7.5 cm (3 inches). According to an estimate, the useful range of pressure differential is probably from 0.25 to 500 grams per square centimetre (0.1 to 200 inches of water column). It is expected that those cathodes utilizing atmospheric pressure or where the gas compartment pressure is not allowed to exceed atmospheric pressure would have a lifetime less than the 1240 hours of Example 2, for instance. It should be noted, however, that all the Examples give the results of tests using NaOH electrolyte only. Chlor-alkali cells were not used, since porous cathodes are not in commercial use as yet. All the above-described tests were conducted at 0.15 ampere per square centimetre (1 ampere per square inch) which was selected for test purposes only for standardization and should not be considered a maximum possible value. It is expected that current densities of the range of 0.3 amperes per square centimetre (2 amperes per square inch) or higher can be used. The tests given in Examples 1-3 were conducted at 60°C, this temperature being chosen simply as a convenient temperature for which standardization can be established.

## Claims

1. A method for operating a chlor-alkali electrolytic cell having an anode compartment, a cathode compartment divided from the anode compartment by a separator and an oxygen compartment divided from the cathode compartment by an oxygen electrode, which method comprises feeding an alkali metal halide solution to the interior of the anode compartment, feeding an aqueous alkaline solution to the interior of the cathode compartment, feeding a gas containing molecular oxygen to the interior of the oxygen compartment, applying an electrical potential between the cathode and the anode, removing halogen gas from the anode compartment, removing alkali metal hydroxide from the cathode compartment and removing an oxygen-depleted gas from the oxygen compartment, characterised in that the gas containing molecular oxygen is depleted of carbon dioxide and humidified and it is fed to the oxygen compartment at a positive gauge pressure in the range from 0.25 to 500 grams per square centimetre (0.1 to 200 inches of H₂0) and so as to provide a total flow rate in excess of the theoretical stoichiometric amount of oxygen necessary for the reaction.

2. A method according to claim 1, wherein the total flow rate is in the range from 1.5 to 21 times the theoretical stoichiometric amount of oxygen.

3. A method according to claim 2, wherein the total flow rate is in the range from 1.5 to 5 times the theoretical stoichiometric amount of oxygen.

4. A method according to any of claims 1 to 3, wherein the positive gauge pressure is in the range from 5 to 250 grams per square centimetre (2 to 100 inches of H₂0).

5. A method according to claim 4, wherein the positive gauge pressure is in the range from 100 to 200 grams per square centimetre (40 to 80 inches of H₂0).

6. A chlor-alkali electrolytic cell for the -production of chlorine and alkali metal hydroxide, comprising an anode compartment for containing an anolyte comprising an alkali metal chloride, a cathode compartment for containing a catholyte comprising an alkali metal hydroxide, a separator dividing the cathode compartment from the anode compartment, an oxygen compartment for receiving an oxygen-containing gas, means for controlling the moisture content of the oxygen-containing gas, means for controlling the total flow-rate of the oxygen-containing gas within the oxygen compartment, an oxygen electrode dividing the cathode compartment from the oxygen compartment, means for removing chlorine from the anode compartment, means for removing alkali metal hydroxide from the cathode compartment, means for supplying alkali metal chloride to the anode compartment and means for supplying electrolyzing electrical energy to the anode and the cathode, characterised in that the cell includes means for controlling the pressure of the oxygen-containing gas within the oxygen compartment.

7. An electrolytic cell according to claim 6, wherein the separator is a diaphragm.

8. An electrolytic cell according to claim 6, wherein the separator is a cation exchange membrane.

9. An electrolytic cell according to claim 8, wherein the cation exchange membrane is a hydraulically-impermeable cation exchange membrane thin film of a fluorinated copolymer having pendant sulphonic acid groups (Nafion).

## Patentansprüche

1. Verfahren zum Betreiben einer Chloralkali-Elektrolysezelle mit einer Anodenkammer, einer Kathodenkammer und dazwischen einer Membran oder ein Diaphragma sowie einer Sauerstoffkammer, die von der Kathodenkammer durch eine Sauers toffel ektrode getrennt ist, dadurch gekennzeichnet, daß man in die Anodenkammer eine Alkalihalogenidlösung, in die Kathodenkammer eine alkalische Lösung und in die Sauerstoffkammer eine Sauerstoff enthaltendes Gas einspeist, zwischen den Elektroden Strom anlegt und aus der Anodenkammer Halogen, aus der Kathodenkammer eine Alkalihydroxidlösung und aus der Sauerstoffkammer ein an Sauerstoff verarmtes Gas ableitet, dadurch gekennzeichnet, daß das sauerstoffhaltige Gas an Kohlendioxid verarmt und befeuchtet ist und in dei Sauerstoffkammer mit einem Überdruck von 0,25 bis 500 g/cm² (3,83 mbar bis 6,78 bar), so daß dadurch das Sauerstoffangebot überstöchiometrisch ist.

2. Verfahren nach Anspruch 1, dadurch gekennzeichent, daß das Sauerstoffangebot die 1,5-bis 21-fache stöchiometrische Menge beträgt.

3. Verfahren nach Anspruch 2, dadurch gekennzeichnet, daß das Sauerstoffangebot die 1,5-bis 5- fache theoretische Menge beträgt.

4. Verfahren nach Anspruch 1 bis 3, dadurch gekennzeichnet, daß man das sauerstoffhaltige Gas mit einem Überdruck von 5 bis 250 g/cm² (2,66 bis 133 mbar) einführt.

5. Verfahren nach Anspruch 4, dadurch gekennzeichnet, daß man das sauerstoffhaltige Gas mit einem Überdruck von 100 bis 200 g/cm² (53,2 bis 106,4 mbar) einführt.

6. Chloralkali-Elektrolysezelle zur Herstellung von Chlor und Alkalihydroxid aufgebaut aus einer Anodenkammer enthaltend eine Alkalichlorid-Lösoung als Anolyt, eine Kathodenkammer enthaltend eine Alkalihydroxid-Lösung als Katholyt, wobei die beiden Kammern durch ein Diaphragma oder eine Membran getrennt sind sowie eine Sauerstoffkammer zur Aufnahme eines sauerstoffhaltigen Gases, Mittel zur Einstellung des Feuchtigkeitsgehalts des sauerstoffhaltigen Gases sowie der gesamten Speisemenge an sauerstoffhaltigem Gas in die Sauerstoffkammer, eine Sauerstoffelektrode zwischen Kathodenkammer und Sauerstoffkammer, eine Chlorableitung aus der Anodenkammer, eine Ableitung für Alkalihydroxidlösung aus der Kathodenkammer, eine Zuführung von Alkalichloridlösung in die Anodenkammer sowie Stromanschlüsse an die Anode und Kathode, dadurch gekennzeichnet, daß die Zelle Mittel zur Einstellung des Druckes des sauerstoffhaltigen Gases innerhalb der Sauerstoffkammer aufweist.

7. Verfahren nach Anspruch 6, dadurch gekennzeichnet, daß die Elekrodenkammern durch ein Diaphragma getrennt sind.

8. Verfahren nach Anspruch 6, dadurch gekennzeichnet, daß die Elektrodenkammern durch eine kationenaustauschende Membran getrennt sind.

9. Verfahren nach Anspruch 8, dadurch gekennzeichnet, daß die kationenaustauschende Membran eine hydraulisch undurchlässige dünne Folie eines fluorierten Copolymeren mit seitlich hängenden Sulfonsäuregruppen ("Nafion") ist.

## Revendications

1. Procédé de conduite d'une cellule d'électrolyse chlore-élément alcalin comportant un compartiment anodique, un compartiment cathodique qu'un séparateur sépare du compartiment anodique, et un compartiment à oyxgène qu'une électrode à oxygène sépare du compartiment cathodique, ce procédé comportant l'apport d'une solution d'un halogénure de métal alcalin à l'intérieur de compartiment anodique, l'apport d'une solution aqueuse alcaline à l'intérieur de compartiment cathodique, l'apport d'un gaz contenant de l'oxygène moléculaire à l'intérieur de compartiment à oxygène, l'application d'un potentiel électrique entre la cathode et l'anode, l'enlèvement du gaz halogène du compartiment anodique, l'enlèvement de l'hydroxyde de métal alcalin du compartiment cathodique, et l'enlèvement d'un gaz appauvri en oxygène du compartiment à oxygène, ce procédé étant caractérisé par le fait que le gaz contenant de l'oxygène moléculaire est appauvri en dioxyde de carbone et humidifié et est envoyé au compartiment d'oxygène sous une pression manométrique positive comprise dans la plage allant de 25 Pa à 50 kPa (0,25 à 500 cm d'eau), et cela de façon à ce que le débit total d'oxygène excède la quantité stoechiométrique théorique d-oxygène nécessaire pour la réaction.

2. Procédé selon la revendication 1, caractérisé par le fait que le débit total est dans la plage allant de 1,5 à 21 fois la quantité stoechiométrique théorique d'oxygène.

3. Procédé selon la revendication 2, caractérisé par le fait que le débit total est dans la plage allant de 1,5 à 5 fois la quantité stoechiométrique théorique d'oxygène.

4. Procédé selon l'une quelconque des revendications 1 à 3, caractérisé en ce que la pression manométrique positive est dans la plage allant de 500 Pa à 25 kPa (5 à 250 cm d'eau).

5. Procédé selon la revendication 4, caractérisé en ce que la pression manométrique positive est dans la plage allant de 10 à 20 kPa (100 à 200 cm d'eau).

6. Cellule chlore-métal alcalin pour produire électrolytiquement du chlore et de l'hydroxyde de métal alcalin, cette cellule comportant un compartiment anodique pour contenir un anolyte qui comporte un chlorure de métal alcalin, un compartiment cathodique pour contenir un catholyte qui comporte un hydroxyde de métal alcalin, un séparateur séparant le compartiment cathodique du compartiment anodique, un compartiment à oxygène pour recevoir un gaz contenant de l'oxygène, des moyens pour commander et/ou contrôler la teneur en humidité du gaz contenant de l'oxygène, des moyens pour commander et/ou contrôler le débit total de gaz contenant de l'oxygène dans le compartiment à oxygène, une électrode à oxygène séparant le compartiment cathodique de compartiment à oxygène, des moyens pour enlever du chlore du compartiment anodique, des moyens pour enlever de l'hydroxyde de métal alcalin du compartiment cathodique, des moyens pour fournir du chlorure de métal alcalin au compartiment anodique, et des moyens pour fournir de l'énergie électrique électrolysante à l'anode et à la cathode, cette cellule étant caractérisée par le fait qu'elle comporte des moyens pour commander et/ou contrôler la pression du gaz contenant de l'oxygène dans le compartiment à oyxgène.

7. Cellule selon la revendication 6, dans laquelle le séparateur est un diaphragme ou membrane.

8. Cellule selon la revendication 6, dans laquelle le séparateur est une membrane échangeuse de cations.

9. Cellule selon la revendication 8, caractérisée par le fait que la membrane échangeuse de cations est une membrane hydrauliquement imperméable, à film mince d'un copolymère fluoré ayant des groupes acide sulfonique y rattachés (NAFION).
